

[54] MAGNESIUM ALLOY FOR DIE CASTING

393,837 6/1933 United Kingdom..... 75/168 D  
516,464 4/1937 United Kingdom..... 75/168 C

[75] Inventors: George S. Foerster, Monmouth Junction; Charles D. Statham, Trenton, both of N.J.

Primary Examiner—C. Lovell

[73] Assignee: N L Industries, Incorporated, New York, N.Y.

## [57] ABSTRACT

[22] Filed: Oct. 1, 1973

A die cast alloy of magnesium has been produced which contains the following ingredients:

[52] U.S. Cl..... 75/168 C; 75/168 B; 75/168 D;  
148/32

5.0% to 20.0% zinc

[51] Int. Cl..... C22c 23/00

0% to 8.5% aluminum

[58] Field of Search ..... 75/168 B, 168 C, 168 D,  
75/168 M, 168 E, 168 F; 148/32; 164/284, 303

0.6% to 6.0% copper

0.05% to 3.0% manganese

0% to 2.0% silicon

the remainder magnesium

## [56] References Cited

all of the percentages expressed on a weight basis.

## UNITED STATES PATENTS

1,341,774 6/1920 Backer..... 75/168 C

## FOREIGN PATENTS OR APPLICATIONS

382,420 10/1931 United Kingdom..... 75/168 C

This alloy has good castability properties coupled with reduced creep extension.

2 Claims, 1 Drawing Figure



SEARCHED JUL 1 1975

3,892,565



## MAGNESIUM ALLOY FOR DIE CASTING

## BACKGROUND OF THE INVENTION

Various magnesium base alloys are described in the art which are useful for die casting. Most of these alloys contain relatively large amounts of aluminum and small amounts of zinc. The instant invention is particularly concerned with the alloys which contain relatively large amounts of zinc and small amounts of aluminum. Although the prior art has prepared alloys containing aluminum and zinc, the prior art has failed to teach the preparation of alloys which have the combination of good castability with a decrease in creep extension.

## SUMMARY OF THE INVENTION

A ductile die cast alloy of magnesium has been prepared comprising aluminum, zinc, copper and manganese with the optional addition of silicon, the balance being magnesium, said alloy having an aluminum and zinc composition by weight which falls within the composition range represented by the pentagon shaped area A, B, C, D and E and bounded by the straight lines AB, BC, CD, DE and EA of the graph in the appended drawing, and containing in addition from 0.6 percent to 6.0 percent copper and from 0.05 percent to 3.0 percent manganese, the balance magnesium.

Compositions of aluminum and zinc represented by the area covered by the pentagon ABCDE correspond in general to the range of zinc in the alloy from 5.0 percent to 20.0 percent and aluminum from 0 percent to 8.5 percent. The alloys also contain copper in amount from 0.6 percent to 6.0 percent, manganese in amount from 0.05 percent to 3.0 percent, the balance being magnesium all of the percentages expressed on a weight basis.

The pentagon is bounded by straight lines connecting the following points:

|   | Zn   | Al  |
|---|------|-----|
| A | 5.0  | 8.5 |
| B | 10.0 | 8.5 |
| C | 20.0 | 0.0 |
| D | 10.0 | 0.0 |
| E | 5.0  | 4.0 |

## DESCRIPTION OF THE DRAWING

Magnesium based alloys containing zinc and aluminum which fall within the compositions contemplated by the instant invention are shown in the drawing. The drawing represents the diagram of the composition Zn + Al defined by the pentagon ABCDE which is bound by the lines AB, BC, CD, DE and EA.

## DESCRIPTION OF THE PREFERRED EMBODIMENTS

Magnesium base alloys which fall within the compositions specified above possess superior properties over those produced by the prior art. These properties include good castability coupled with decreased creep extension without substantially affecting the corrosion resistance, the yield strength and the tensile strength.

It has been discovered that the presence of a small amount of manganese, i.e., at least 0.05 percent, aids in improving the corrosion resistance and creep extension in the alloy. The creep extension expressed in percent was measured on test bars at a tensile loading of

5 kilo pounds per square inch (k.s.i.) for 100 hours at 350°F. The addition of silicon up to 2.0 percent also tends to improve the fluidity and strength.

Alloys which are prepared having zinc contents below the minimum amount specified above have poor castability while alloys prepared having zinc contents above the maximum amounts specified become brittle.

It has also been found that the maximum amount of copper employed preferably should be no more than 0.5 times the zinc content.

In order to describe the instant invention in more detail, the following examples are presented:

## EXAMPLES 1-7

15 Several magnesium base alloys containing various amounts of zinc, aluminum, manganese and copper were prepared. All of these alloys fell within the zinc and aluminum pentagon ABCDE.

The compositions of the various alloys are recorded 20 in Table 1.

The various alloys were produced by melting commercial grade magnesium at 1300°F under halide flux cover. Zinc, aluminum and copper chunks in the desired proportions as shown in the Table were added to the molten magnesium to dissolve the chunks. The manganese was added as manganese chloride. The so-prepared melts were then each die cast into a heated die at 500°F and 8,000 psi, having a cavity configuration of an ASTM E8-68, FIG. 1e, 2 inch gauge length 30 test bar. These bars were then tested for yield strength - ultimate tensile strength, and percent creep at a tensile loading of 5 k.s.i. for 100 hours at 350°F. All data are recorded in the table.

For comparative purposes, alloys having compositions 35 which contain less than 0.6 percent copper but which lie inside the pentagon ABCDE were prepared as controls and their results were compared with the above examples.

These compositions and their properties are also recorded in the table as Controls A-D.

It has also been discovered that the presence of manganese in amounts from 0.05 percent to 3.0 percent is effective in increasing the corrosion resistance and tends to improve the creep resistance.

45 The corrosion resistance of these alloys was determined as follows:

Standard die-cast tensile bars were cut in half to obtain corrosion test specimens 4-1/2 inches long with a major diameter of 3/8 inch. After cleaning to remove 50 surface contamination, the specimens were weighed and then partially submerged in aerated 3% NaCl solution saturated with MgO (pH 10.3) for three days at room temperature. The specimens were mounted vertically through holes in a plastic sheet which served as the cover of the test vessel. Approximately 80% of the specimen length was submerged. At the end of the test period, the products were removed by immersing the specimens in a solution containing 20% CrO<sub>3</sub> and 1% AgNO<sub>3</sub>. The final weights were then determined and the average corrosion rates calculated from weight loss, submerged area, and test duration.

60 It should be noted that the creep extensions of Examples 1-6 were all less than all of the corresponding controls which contained less than 0.6 percent copper. In addition to improved creep resistance, these alloys also possess satisfactory corrosion resistance. From the above examples, it has clearly been shown that alloys

of magnesium containing amounts of zinc and aluminum which fall within the specified composition range shown in the pentagon ABCDE and containing the specified amounts of copper and manganese, possess superior resistance to creep coupled with good castability and adequate corrosion resistance when the copper content is held within the specified limits.

While this invention has been described and illustrated by the examples shown, it is not intended to be strictly limited thereto, and other variations and modifications may be employed within the scope of the following claims.

ing of zinc, aluminum, copper, manganese, silicon and magnesium, said zinc and aluminum present in amounts which fall within the pentagon ABCDE in the accompanying drawing defined by the lines AB, BC, CD, 5 DE and EA, said alloy also containing copper in amount from 0.6 percent to 6.0 percent, manganese in amount from 0.05 percent to 3.0 percent, silicon in amount from 0.0 percent to 2.0 percent, the remainder magnesium, all of the percentages expressed on a 10 weight basis.

## 2. A die cast alloy of magnesium according to claim

TABLE

|            | COMPOSITION |      |      |     | AS CAST (Room Temperature) |                                   |         |                         |      |
|------------|-------------|------|------|-----|----------------------------|-----------------------------------|---------|-------------------------|------|
|            | %Al         | %An  | %Cu  | %Mn | Yield Strength<br>Ksi      | Ultimate<br>Tensile Strength<br>% | % Creep | Corrosion<br>Resistance |      |
| Control A  | 0.0         | 15.9 | 0.3  | 2.1 | 26.5                       | 33.2                              | 3.0     | 4.84                    | 0.7  |
| Example 1  | 0.0         | 15.9 | 1.1  | 2.1 | 27.9                       | 37.4                              | 4.5     | 3.1                     | 0.69 |
| Example 2  | 0.0         | 15.9 | 3.2  | 2.1 | 26.8                       | 34.3                              | 4.0     | 1.21                    | 0.96 |
| Control B  | 4.2         | 12.2 | 0.35 | 0.3 | 28.1                       | 37.5                              | 3.9     | .62                     | 0.17 |
| Example 3  | 4.2         | 12.2 | 1.1  | 0.3 | 28.2                       | 35.7                              | 2.6     | .36                     | 0.26 |
| Example 4  | 4.2         | 12.2 | 3.1  | 0.3 | 29.6                       | 37.0                              | 2.0     | .32                     | 0.36 |
| Control C  | 7.1         | 6.6  | 0    | .21 | 25.2                       | 34.2                              | 2.6     | 2.47                    | —    |
| Example 5  | 7.1         | 6.6  | 1.0  | .21 | 27.8                       | 37.9                              | 4.2     | 1.48                    | 0.22 |
| Example 6  | 7.1         | 6.6  | 3.2  | .21 | 29.2                       | 37.4                              | 2.1     | 0.50                    | 0.52 |
| <u>%Si</u> |             |      |      |     |                            |                                   |         |                         |      |
| Control D  | 3.8         | 9.6  | 0    | .14 | 1.0                        | 25.6                              | 34.1    | 2.8                     | 0.90 |
| Example 7  | 3.8         | 9.6  | 0.95 | .14 | 1.0                        | 27.3                              | 36.6    | 3.8                     | 0.24 |
|            |             |      |      |     |                            |                                   |         |                         | 0.20 |

We claim:

1. A die cast alloy of magnesium having good castability and improved creep extension, said alloy consist-

1 in which the copper content of said alloy should be no more than 0.5 times the zinc content.

\* \* \* \* \*